

## UNITED STATES PATENT OFFICE

2,257,359

WATER-CONTAINING LUBRICANT FOR  
COMPOSITION BEARINGS

Robert C. Williams, Columbus, Ohio, assignor to  
The Ironsides Company, Columbus, Ohio, a corporation of Ohio

No Drawing. Application May 5, 1939,  
Serial No. 272,015

## 4 Claims. (Cl. 184—1)

This invention relates to lubricants and more particularly to lubricants of the type wherein water is the predominating ingredient, the remaining ingredients being present in proportions of less than 10% by weight.

In a more specific aspect, the present invention is concerned with the provision of an improved lubricant and/or coolant for composition bearings. The use of composition bearings, typified by molded or laminated phenol-formaldehyde resin bearings, is common in rolling mill practice. Water, in lieu of a petroleum lubricant, is quite widely used as a coolant for these bearings, since the latter will not tolerate as much heat as metallic bearings without suffering marked deterioration. Water, so employed, serves as a lubricant in addition to its cooling function.

To function advantageously, however, best results are obtained when the water is fully and equally distributed over the bearing surfaces. Bearing surfaces, composed of phenol-formaldehyde resins, and other related condensation products, are not readily and completely "wet" by water. This is evident by the way water gathers in the form of capillary beads on the surfaces of such materials.

It is an object of the present invention to improve the lubricating and/or cooling powers of water, when the latter is employed in the capacity set forth, by the addition thereto of suitable spreading or "wetting" agents. Many of these so-called "wetting" agents are now available on the open market under various trade names and certain of which I have found suitable for the purposes of the present invention. The addition of minor percentages of these agents enable water to spread evenly over the rubbing surfaces of the bearings, providing the latter with liquid protection of such nature that relatively low rotational speeds of the rotating part of the bearing, and high unit pressures, may be successfully withstood without overheating.

By way of examples of wetting or spreading agents which I have found suitable for the ends herein sought are the following:

(1) R—CO<sub>2</sub>Na—where R represents the fatty alkyl groups. Ordinary soap, such as sodium oleate, is an example of this type.

- 5 (2) R—SO<sub>4</sub>Na—fatty alcohol sulphates are examples of this type.  
3 (3) R'Ar—SO<sub>3</sub>Na—where R' is a primary or secondary non-fatty alkyl group and Ar an aryl or aromatic group. The sodium salt of isopropyl naphthalene sulphonic acid is an example of this type of wetting agent.  
10 (4) R'—CHSO<sub>4</sub>Na—the so-called "Tergitol" compounds, namely, sodium secondary-alcohol sulphates.  
(5) Common sulphonated oils, such as castor oil.  
(6) R—CONHC<sub>2</sub>H<sub>4</sub>SO<sub>4</sub>Na (sulphated fatty acid amides).  
15 (7) R—COOC<sub>2</sub>H<sub>4</sub>SO<sub>4</sub>Na (sulphated fatty acid esters).  
(8)



(sulphonated esters of alcohols and dibasic acids)



(sulphated esters of higher alcohols and dibasic acids)

30 The general characteristic of suitable wetting agents is the existence in the molecule of a polar group, which is strongly hydrophilic, and a non-polar group, generally of a hydrocarbon nature, as represented by R, R' or Ar above.

Certain wetting agents, such as those set forth 35 in most of the examples above, are effective in resisting the action of hard water and, also, tend to prevent the precipitating action of hard water on soap when used in connection with soap. It is within the purview of the invention to use these 40 wetting agents in conjunction with soap, oil-in-water emulsions and alone. The amount of the wetting agent employed is usually very low, as disclosed in the following tables. In use, the lubricant or coolant is circulated in a closed system 45 of which the bearing is a part, so that loss of the agent is minimized.

In testing the lubricants forming the present invention, a phenol-formaldehyde resin type of bearing was held against a steel rotor in a Timken lubricant tester. Many such tests disclosed that

the power consumption when a wetting agent was employed was much less than when water was used alone. Results of certain of such tests are to be found in the following table:

| Lubricant                                                                                           | Working load                                          | Rotor<br>R. P. M.                                | Power<br>required<br>to operate<br>machine |
|-----------------------------------------------------------------------------------------------------|-------------------------------------------------------|--------------------------------------------------|--------------------------------------------|
| Water, obtained from<br>municipal mains, Co-<br>lumbus, Ohio.                                       | 20 lbs. on lever<br>(12,500 lbs. per<br>square inch). | 800 ft. per<br>minute at<br>rubbing<br>surfaces. | Watts,<br>860                              |
| Water, as above, con-<br>taining:                                                                   |                                                       |                                                  |                                            |
| 3.5% potash soap                                                                                    | do                                                    | do                                               | 560                                        |
| 1.75% potash soap                                                                                   | do                                                    | do                                               | 520                                        |
| .24% potash soap,                                                                                   | do                                                    | do                                               | 510                                        |
| 2.16% fat.                                                                                          |                                                       |                                                  |                                            |
| 0.5% Tergitol 4 (a so-<br>dium secondary alco-<br>hol sulphate).                                    | do                                                    | do                                               | 740                                        |
| .1% to .2% Orvus W—<br>a paste comprising a<br>fatty alcohol sulphate<br>of the $R-SO_4Na$<br>type. | do                                                    | do                                               | 750                                        |
| .1% Santo-Merse No. 3<br>(a substituted aromatic<br>sulphonic acid<br>salt).                        | do                                                    | do                                               | 760                                        |
| .2% to 4% sulfonated<br>castor oil (75%<br>strength). .1% Santo-<br>Merse No. 3.                    | do                                                    | do                                               | 730                                        |

The above percentages of the various ingredients given are by weight. This is true in the balance of the specification and claims, unless otherwise specified. In conducting the above tests, the temperatures of the various lubricants were always well within the safe limits of bearing operation.

Another important group of wetting agents satisfactory for the purpose of lubricating composition bearings is that of "water-soluble" oils. Such oils contain dispersing compounds. Certain petroleum oils are readily soluble in these compounds and the latter are, in turn, soluble in water. Examples of such dispersing compounds are butyl alcohol or certain soaps, among which may be mentioned triethanolamine soap. Such a soluble oil is homogeneous in appearance and is spontaneously emulsified as an oil-in-water emulsion on being added to water. There are several types of these soluble oils, the types being differentiated by the dispersing compound employed. Typical of such a composition is the following:

|                                                 | Per cent |
|-------------------------------------------------|----------|
| Paraffin oil (Saybolt vis. 100 sec. at 100° F.) | 76.2     |
| Triethanolamine                                 | 7.8      |
| Oleic acid                                      | 16.0     |
|                                                 | 100.0    |

The above preparation may be added to water to form the internal phase of the resulting emulsion, in proportions of less than 5% by weight to the water used.

I am aware of the fact that composition bearings composed of phenol-formaldehyde condens-

sation products have been lubricated with water but so far as I am aware, the water has not been modified by the addition of minor percentages of wetting agents thereto. Also, in the lubrication of composition bearings, soaps have been added to glycerin, but in this class of lubricants, the water employed, if any, has been but a minor ingredient. In the lubricants or coolants of the present invention, water predominates and but a very small percentage of the wetting agents is used.

It will be understood that my improved lubricant is adapted to bearings generally and especially composition bearings formed from any of the so-called plastics which lend themselves to bearing construction.

A further advantage gained by the use of my improved lubricant is the protection of the bearing by the film left on the bearing surface when starting up a mill following a shut-down. Present practice is to coat the roll necks with grease or oil to prevent seizure taking place during the shut-down. The use of my improved lubricant makes this unnecessary.

What is claimed is:

1. The method of lubricating composition bearings of the phenol-formaldehyde resin type, comprising applying to the journal surfaces of such a bearing during active use of the latter a liquid composed principally of water and having uniformly dispersed therein minor percentages of a wetting agent, said agent being a water miscible compound of the class represented by the formula  $R-SO_x-M$  wherein  $R$  represents a non-polar group of a hydrocarbon nature from the group consisting of fatty alkyls, primary and secondary non-fatty alkyls, and aryls;  $SO_x$  represents a strongly hydrophilic polar group from the class consisting of sulfates and sulfonates; and  $M$  represents an alkali metal.

2. The method of lubricating and cooling composition bearings of the synthetic resin type which are not readily "wet" by water which comprises the step of applying to the journal surfaces of such a bearing during active use thereof an aqueous lubricant, said lubricant being composed primarily of water and containing as an essential component a wetting agent dispersed therein of the class represented by the formula  $R-SO_x-M$  wherein  $R$  represents a non-polar group of a hydrocarbon nature from the group consisting of fatty alkyls, primary and secondary non-fatty alkyls, and aryls;  $SO_x$  represents a strongly hydrophilic polar group from the class consisting of sulfates and sulfonates; and  $M$  represents an alkali metal.

3. The method as set forth in claim 2 in which the wetting agent is a sulfated fatty hydrocarbon derivative.

4. The method as set forth in claim 2 in which the wetting agent is a sulfonated hydrocarbon derivative.

ROBERT C. WILLIAMS.